

Oct. 20, 1931.

T. H. FROST

1,827,870

FINE EDGED BLADE

Filed May 24, 1930



Fig.1.



Fig.2.

INVENTOR.

Thomas H. Frost.

by M.W. Murray, atty

## UNITED STATES PATENT OFFICE

THOMAS H. FROST, OF CAMBRIDGE, MASSACHUSETTS

## FINE EDGED BLADE

Application filed May 24, 1930. Serial No. 455,366.

This invention relates to fine edge blades, such for example, as safety razor blades of the thin flexible type which are adapted for use in holders wherein they are clamped for support. In a broad aspect my invention consists in a blade of a ferrous nitridable alloy, nitrided in areas adjacent to and including its cutting edge. I have discovered that blades thus characterized possess an edge holding quality which gives them great value as cutting instrumentalities both from the stand-point of smooth-cutting and in respect to the life of the blade.

The material I employ in the construction of the novel blade of my invention is an alloy of steel containing a substantial amount of aluminum, usually combined with chromium or molybdenum or tungsten and which may be hardened by a process of nitriding, that is to say, by introducing nitrogen into, or causing it to combine with the alloy. One suitable alloy of this type is known under the name "nitr alloy" by which it is commonly designated. When this metal is exposed to ammonia fumes under conditions of high temperature it becomes nitrided upon its surface and to a slight distance below its surface and is thereby rendered extremely hard and brittle. Attempts to use this material in the

manufacture of blades heretofore have been unsuccessful partly on account of the fact that a contraction or expansion takes place in the nitriding operations which warps or distorts the blank to an extent rendering sharpening difficult or impossible. In accordance with an important feature of my invention I confine the nitriding of the blank to areas adjacent to and including the cutting edges of the blade. This permits expansion of the portions of the blade including the cutting edges by internal adjustment of the blank in its unnitrided areas with the result that the critical portions of the blade are preserved in a flat condition without distortion.

In applying my invention to a safety razor blade I provide the blank with a central longitudinal slot substantially co-extensive in length with the cutting edge of the blade and effective to a certain extent in isolating the body of the blade from the portion including

its cutting edge or, in the case of a double edged blade, isolating from each other the two portions in which the cutting edges are formed. In a blade provided with a slot of this character the end portions which lie beyond the cutting edge of the die are unnitrided and are accordingly soft in character so that any change in the shape of the nitrided portions may be readily absorbed without distorting the blade as a whole.

These and other features of the invention will be best understood and appreciated from the following description of a preferred embodiment thereof selected for purposes of illustration and shown in the accompanying drawings, in which—

Fig. 1 is a plan view of the blade upon an enlarged scale, showing certain end areas protected for nitriding the process,

Fig. 2 is a similar view of the finished blade.

The material employed in producing blades in accordance with my invention may be any nitridable ferrous alloy having the characteristics best suited for the particular type of edged tool required. Nitr alloy of either of the following analyses has been found satisfactory for the manufacture of razor blades:

| Element         | Analysis A | Analysis B |
|-----------------|------------|------------|
| Carbon.....     | .36        | .23        |
| Manganese.....  | .51        | .51        |
| Silicon.....    | .27        | .20        |
| Aluminum.....   | 1.23       | 1.24       |
| Chromium.....   | 1.49       | 1.58       |
| Sulphur.....    | .010       | .011       |
| Phosphorus..... | .013       | .011       |
| Molybdenum..... | .18        | .20        |

In manufacturing the blade herein shown a blank of nitr alloy is first prepared by punching from strip stock or otherwise. This may be used as received from the producer or after it has been heat-treated to refine the micro-structure of the alloy, but in either case the sheet nitr alloy is in such condition that it may be readily blanked out. The blank thus produced is of the thickness and outline desired in the finished blade and, as herein shown, has corner recesses defining a central elongated portion. The blank is

also internally apertured, being provided with an elongated slot 4 having a central aperture 6 for the stud of the razor holder.

As already explained, I do not desire to nitride the entire area of the blade blank but wish to preserve an area at each end of the blade in unnitrided condition. To this end I coat a fan-shaped area at each end of the blade with a protective material, such as a paste of stannic oxide 8 in water or glycerine, which in the subsequent nitriding process is reduced to metallic tin, coating the blank and rendering it impervious to the action of the ammonia fumes. The outline of the unnitrided area may be selected as desired but as herein shown each area is generally fan-shaped and includes one end of the slot 4 and an elongated end portion of the blade.

Having prepared the blank as above outlined it is then heated in a furnace in the presence of ammonia gas at a temperature sufficiently high to insure carrying out the nitriding operation. In some cases a temperature of 930-950° F. will be found suitable but I have secured entirely satisfactory results by treating the blank at a somewhat higher temperature. This results in a deeper penetration of the nitriding effect and a somewhat softer resulting material than is produced at lower temperatures. The nitriding operation may be satisfactorily carried out at a temperature of 950° F. in an interval of two hours or somewhat less, while at a temperature of 1150° F. the operation may be complete in as short an interval as five minutes.

The temperature and time used for the nitriding of razor blades may be considered as determining the shaving characteristics of the finished blade. For example, a blade nitrided for two hours at 950° F. when finish sharpened in the ordinary manner gives a sharp but fairly rough edge. If the nitriding operation be carried out at 1150° F. for twenty minutes, the penetration into, or addition of nitrogen to the exposed metal at the higher temperature being more rapid and also resulting in a softer finished product, the blade when finish sharpened in the same manner as the first blade shows a sharp but smooth edge. Some shavers prefer smooth edged blades and some prefer rough edged blades and these different types of edges may be procured in accordance with my invention by variation of the nitriding temperature to suit the conditions desired.

The length of time of nitriding at any given temperature determines the depth of the nitrided case. This case must be deep enough to allow for any material which may be taken off during finish sharpening operation. The two specified temperatures and times have been found to be satisfactory. It is evident of course that a compromise between a smooth and a rough edge may be ob-

tained by nitriding at a temperature between 1150° F. and 950° F. and for a time long enough to secure the necessary depth of case. Temperatures higher and lower than those above specified may be used with a corresponding decrease or increase in the time necessary for satisfactory nitriding.

In the nitriding process, as already explained, there is an appreciable internal adjustment of the alloy being treated in a blank of the form shown in Fig. 1. This may take place independently in each side portion of the blank separated by the slot 4, and since the end areas remain in a relatively soft condition and substantially unaffected by the nitriding process this adjustment will be absorbed in them without objectionable distortion of the blade as a whole.

In carrying out the nitriding process the two side portions of the blade are converted into an extremely hard material having edge holding properties of a degree heretofore unattainable. The blade may be then completed by finish grinding its opposite longitudinal edges in the usual manner to form the sharpened nitrided cutting edges 12.

Relatively soft materials such as nitr alloy of the analyses given above, have a tendency to form a "feather" when ground to a fine edge. In the manufacture of razor blades it was found that this tendency to "feather" caused objectionable inequalities in the finished edge. In producing the novel blade of my invention this objection is avoided since the finish grinding operation is carried out upon the material hardened by the nitriding process. The material removed in grinding therefore comes off smoothly and leaves the blade in excellent condition for honing and stropping.

While I have shown my invention as embodied in a safety razor blade it will be understood that it may be applied with advantage to fine edged tools of all descriptions and I have particularly in mind surgeons' knives, pocket knives, cutting edges and cutlery for general purposes.

Having thus described my invention, what I claim as new and desire to secure by Letters Patent of the United States is:—

1. A thin flexible blade of nitr alloy, nitrided in an area adjacent to and including its cutting edge.
2. A flexible fine edged blade of nitr alloy, nitrided in an area adjacent to its cutting edge and having unnitrided supporting portions.
3. A fine edged blade of nitr alloy, nitrided in an area which includes its cutting edge and having a slot parallel to its cutting edge which defines one edge of the nitrided area.
4. A fine edged blade of nitr alloy, nitrided in an area which includes its cutting edge, having a slot substantially parallel to said

edge, and unnitrided areas merging into the nitrided area at either end of the slot.

5. A safety razor blade comprising a thin flexible wafer of nitr alloy internally apertured and nitrided in areas adjacent to its cutting edge.

19 6. A safety razor blade comprising a thin flexible wafer of nitr alloy having a nitrided area including its cutting edge and an unnitrided area merging into the same and permitting expansion of the nitrided area without deformation of the cutting edge.

15 7. A safety razor blade comprising a thin flexible wafer of nitr alloy with its opposite longitudinal edges sharpened for cutting and a central longitudinal slot, and being nitrided in areas coextensive with said slot.

20 8. A safety razor blade comprising a thin flexible wafer of nitr alloy, the blade being nitrided and sharpened at opposite edges and having a central slot of substantially the same length as said edges and unnitrided end areas beyond said cutting edges.

25 9. A safety razor blade comprising a thin flexible wafer of nitr alloy with opposite cutting edges and a central internal slot, the edge areas of the wafer being nitrided and being connected by unnitrided end portions, whereby the nitriding of the edge areas may 30 be carried out without distortion of the blade as a whole.

35 10. A safety razor blade made of a nitridable alloy and comprising a flat body portion of substantially uniform thickness and an acutely tapered cutting edge portion integral therewith, said blade being nitrided in an area adjacent to and including its cutting edge and having an area with an unnitrided surface merging into the same.

40 11. A safety razor blade made of a nitridable alloy and comprising a thin flat body portion of substantially uniform thickness and an acutely tapered cutting edge portion integral therewith, said blade being nitrided 45 in an area adjacent to and including its cutting edge.

Signed at Boston, Massachusetts, this 23rd day of May, 1930.

THOMAS H. FROST.